

Patented Jan. 5, 1937

2,066,506

## UNITED STATES PATENT OFFICE

2,066,506

## FUEL

Clifford A. Woodbury, Media, Pa., and Walter E. Lawson, Wilmington, Del., assignors to E. I. du Pont de Nemours & Company, Wilmington, Del., a corporation of Delaware

No Drawing. Application October 13, 1932,  
Serial No. 637,670

## 4 Claims. (Cl. 44—9)

This invention relates to improvements in compression ignition fuels and it particularly relates to the use of novel ignition accelerators for the said fuels.

5 One object of this invention relates to improvements in Diesel engine fuels and particularly in fuels adapted for use in high-speed compression ignition engines whereby to obtain a reduction of the delay period between the injection and the ignition of the fuel oil, a reduction in the ignition temperature of the fuel oil and/or a lowering of the compression ratio of the engine. A specific object relates to compression ignition fuels containing a nitrate of a polyhydric alcohol derivative, said derivative containing one or more solubilizing groups. A more specific object relates to compression ignition fuels containing as an ignition accelerator a polynitrate alkyl ester containing a solubilizing group. Other objects of 10 the invention will become apparent from the following description.

In accordance with the present invention, it has been found that when nitrates of polyhydric alcohols so modified as to render them soluble in the fuel oil are added to the fuel oil there is obtained a reduction in the delay period between injection and ignition of the fuel oil. This phenomenon is accomplished by a lowering of the ignition temperature of the fuel oil and/or a lowering of the compression ratio in the compression engine required to ignite the fuel.

The following table illustrates examples of nitrates of polyhydric alcohol derivatives containing solubilizing groups which may be used in accordance with the practice of the invention. This table also illustrates the effect of the use of these esters on the fuel oil characteristics. The properties of the doped or modified fuel oil are compared with those of unmodified fuel oil, the same quality of fuel oil being used in all of the examples.

| 45 | Composition<br>fuel   | Accelerator                                | Second<br>delay<br>at 514°<br>C. | Min-<br>imum<br>ignition<br>temp. | Min-<br>imum<br>com-<br>pression<br>ratio |
|----|-----------------------|--------------------------------------------|----------------------------------|-----------------------------------|-------------------------------------------|
|    | Fuel oil.....         | Propylene glycol dinitrate.                | 0.94                             | 500                               | 9.5                                       |
|    | Fuel oil+5% by<br>wt. | 0.20                                       | 300                              | 9.4                               |                                           |
| 50 | Fuel oil+5% by<br>wt. | 1, 3 butylene glycol<br>dinitrate.         | 0.12                             | 300                               | -----                                     |
|    | Fuel oil+5% by<br>wt. | Dimethylidimethylol-<br>methane dinitrate. | 0.12                             | 300                               | 8.8                                       |
|    | Fuel oil+5% by<br>wt. | Dinitrochlorohydrin.                       | 0.17                             | 300                               | 9.2                                       |
|    | Fuel oil+5% by<br>wt. | Ethylenechlorohydrin<br>nitrate.           | 0.12                             | 300                               | -----                                     |
| 55 | Fuel oil+5% by<br>wt. | Monooethyltin dinitrate                    | 0.11                             | 275                               | -----                                     |

The method of test for determining the ignition delay and minimum ignition temperature consisted in injecting the fuel oil into air at atmospheric pressure into a heated chamber. The

ignition delay is the elapsed time between injection and ignition of the fuel. The minimum ignition temperature is the lowest temperature at which a majority of a series of samples injected into the chamber ignite. The minimum compression ratio was determined according to the method described by Pope and Murdock in the Society of Automotive Engineers Journal, Transactions, pages 136-142 for March 1932.

The compounds suitable for use according to 10 the present invention all contain at least one nitrate group. The most generally satisfactory alkyl nitrates are those which contain at least two nitric ester groups. These nitrate esters are modified by the inclusion in their molecules of radicals which confer upon them the property of dissolving to a substantial extent in fuel oil of the type used in Diesel engines. Examples of solubilizing groups forming radicals in the said esters are halogen, aliphatic hydrocarbon, acyloxy, alkoxy and aryloxy radicals. In the case of the polynitrate esters, hydrocarbon radicals, both aliphatic and aromatic, increase the solubility of the compounds in the fuel oil. The compounds listed in the table described above are merely illustrative, the nitrate esters being capable of considerable variation from the specific esters listed above. For purposes of simplicity the nitric esters of polyhydric alcohols which can be used in the practice of the present invention are divided into 15 the following three general classes:

1.  $RHC_2-(CHONO_2)_nH$  where  $n$  is 2 or more and  $R$  is hydrogen, or a hydrocarbon radical.
2.  $RCH_2-(CHONO_2)_xH$  where  $x$  may be any small whole number and  $R$  may be chosen from 25 the class consisting of halogen, acyloxy, alkoxy, aryloxy, and a hydrocarbon radical containing a nitric ester group.

3.



40

where  $R$  may be a hydrocarbon radical and  $R_1$  may be chosen from groups consisting of hydrocarbon, nitro, and nitric ester of methylol radicals.

Specific examples of compounds of formula 1 comprise 1,2-propylene glycol dinitrate, 1,2-butylene glycol dinitrate, 1,2-ethylene glycol dinitrate, and 3-phenyl-1,2-propylene glycol dinitrate.

Specific examples of compounds of formula 2 comprise 1,3-butylene glycol dinitrate, monoethyl ether of glycerol dinitrate (monoethyltin dinitrate), monoacetic acid ester of glycerol dinitrate (monoacetyl dinitrate), monophenyl ether of glycerol dinitrate, glyceryl monochloride dinitrate (dinitro chlorhydrin), monoethyl ether of ethylene glycol nitrate, ethylene chlor-

50

55

60

hydrin nitrate, ethylene bromhydrin nitrate, monophenyl ether of ethylene glycol nitrate, and monoacetic acid ester of ethylene glycol nitrate.

Specific examples of compounds of formula 3 5 comprise dimethyldimethylolmethane dinitrate, ethyltrimethylolmethane trinitrate, methyltrimethylolmethane trinitrate, and nitromethyldimethylolmethane dinitrate.

All of the above compounds are included under 10 the generic term "a nitrate of a polyhydric alcohol derivative, said derivative containing a solubilizing group".

The advantages of the use of these accelerators 15 in fuel oil for compression ignition engines are:

1. Elimination of knocking and rough-running by decreasing the ignition lag.

2. Reduction of engine wear by removing the cause of knocking and roughness.

3. Easier starting. The reduced spontaneous 20 ignition temperatures of the doped oil enable it to ignite much more easily when starting from cold.

4. Improved exhaust. Owing to the more complete combustion the exhaust is cleaner especially at higher speeds. No harmful constituents are introduced into the exhaust gases by the combustion of the dope.

5. Possibility of use of inferior fuels. By the 25 addition of dope, low grade fuels, at present quite unsuitable for compression ignition engines, can be rendered equal or superior to high grade undoped fuels.

6. Nature of dope. The dope has a neutral reaction, is non-toxic and soluble in the oil.

35 7. Improvements in engine design. Reduced engine stresses, resulting from the more gradually applied piston pressures, should make for lighter scantlings while the more readily ignited and rapidly burning fuel should render possible 40 the construction of smaller and faster running engines.

8. Increased power and reduced fuel consumption. The improved combustion resulting from the explosive action of the dope enables a greater 45 proportion of the air charge to be burnt, and further, as ignition takes place at once, the fuel can be injected during the compression stroke at a smaller crank angle near top dead center.

The advantages of the invention over the prior 50 art result from decreased vapor pressure of the nitrates of modified polyhydric alcohols. The boiling points of a few compounds used as fuel dopes, including those of the present invention, are given in the following table:

| Dope                            | Boiling point       |
|---------------------------------|---------------------|
| Methyl nitrate.....             | 55° C.              |
| Ethyl nitrate.....              | 87° C.              |
| Propyl nitrate.....             | 110.5° C.           |
| Propylene glycol dinitrate..... | 92° C. at 10 mm.    |
| Dinitrochlorhydrin.....         | 117.5° C. at 10 mm. |

Further advantages are:

1. The increased boiling point prevents the formation of vapor locks in the fuel system of the engine.

2. Elimination of hazard in transportation and 5 storage. The decreased vapor pressures eliminate the possibility of the formation of an explosive, dope-air mixture above the fuel in tank cars or storage tanks.

3. Decrease in objectionable physiological 10 properties. The decreased vapor pressure of the dopes also decreases the physiological effects, such as headaches, which constitute an objection to lower alkyl nitrates.

The above description and examples are to be 15 taken as illustrative only and not as limiting the scope of the invention. Any modification or variation therefrom which conforms to the spirit of the invention is intended to be included within the scope of the claims. 20

We claim:

1. A compression ignition engine fuel comprising a high boiling fuel oil containing a nitrate of an aliphatic polyhydric alcohol selected from the group consisting of 1,2-propylene glycol dinitrate, 1,2-butylene glycol dinitrate, 1,2-ethylene glycol dinitrate, 3-phenyl-1,2-propylene glycol dinitrate, 1,3-butylene glycol dinitrate, monoethyl ether of glycerol dinitrate, monoacetic acid ester of glycerol dinitrate, monophenyl ether of glycerol dinitrate, glyceryl monochloride dinitrate, monoethyl ether of ethylene glycol nitrate, ethylene chlorhydrin nitrate, ethylene bromhydrin nitrate, monophenyl ether of ethylene glycol nitrate, monoacetic acid ester of ethylene glycol nitrate, dimethyldimethylolmethane dinitrate, ethyltrimethylolmethane trinitrate, methyltrimethylolmethane trinitrate, and nitromethyldimethylolmethane dinitrate. 25 30 35 40

2. A compression ignition engine fuel comprising a high boiling fuel oil containing monoethyl ether of glycerol dinitrate.

3. A compression ignition fuel comprising a high boiling fuel oil containing 1,2-propylene glycol dinitrate. 45

4. A compression ignition fuel comprising a high boiling fuel oil containing dimethyldimethylolmethane dinitrate. 50

CLIFFORD A. WOODBURY.  
WALTER E. LAWSON.

Patent No. 2,066,506.

CLIFFORD A. WOODBURY ET AL.

January 5, 1937.

It is hereby certified that error appears in the printed specification of the above numbered patent requiring correction as follows: Page 1, second column, line 32, for "RHC<sub>2</sub>" read RCH<sub>2</sub>; and that the said Letters Patent should be read with this correction therein that the same may conform to the record of the case in the Patent Office.

Signed and sealed this 23rd day of March, A. D. 1937.

[SEAL]

HENRY VAN ARSDALE,  
Acting Commissioner of Patents.